

Dec. 24, 1946.

A. H. WARTH ET AL

2,413,093

FILM-FORMING RESINOUS LINING FOR METAL CONTAINERS

Filed July 20, 1942

Fig. 1.



Fig. 2.



Fig. 3.



Inventors:

Albin H. Warth,  
Iliya F. Bulatkin,  
By Cushman, Durby & Cushman

Attorneys.

## UNITED STATES PATENT OFFICE

2,413,093

FILM-FORMING RESINOUS LINING FOR  
METAL CONTAINERS

Albin H. Warth and Iliya F. Bulatkin, Baltimore,  
Md., assignors to Crown Cork & Seal Company,  
Inc., Baltimore, Md., a corporation of New York

Application July 20, 1942, Serial No. 451,620

4 Claims. (Cl. 220—64)

1

This invention relates to containers for maintaining the original quality and freshness of foods and beverages, particularly beer and ale.

A most significant feature of the present invention is the provision of a container having a lining which is stable to such delicate products as beers and ales, being acid resistant and containing no metallic elements that might react with the proteins in such beers and ales. This container is provided with a wax coating superposed upon the lining at the bottom seal only instead of the usual overall wax coating. The wax coating at the seam is assurance against any possibility of rusting and also enhances the seal at the seam.

A container having a construction of this character precludes the necessity of using aluminum coated steel and which moreover must have an overall coating of wax to prevent bleaching of the contents such as beer by the aluminum. In other words, the lining of the container of this invention does not exert this objectionable effect and hence a wax coating for the entire container body as generally used is now obviated.

The primary object of the invention is to provide a container having a lining which is non-absorbent as regards the contents. Thus, the principles contributing to the flavor, aroma and color of such a delicate product as beer remain unimpaired through long periods of storage.

A coating comprising asphalt and gilsonite has heretofore been suggested, but it was found that such coatings tend to absorb the taste and flavor of beverages, such as beer, and are, therefore, objectionable. Attempts have been made to overcome this deficiency in such coatings by adding flavor-imparting ingredients, such as lupulin, but such expedients have not been found to be satisfactory.

Linings formed from synthetic resin varnish-like materials have also been used, but have been found to be objectionable for various reasons.

Our invention resides in the discovery that "Aruba" resin when incorporated in a lining having a suitable non-volatile, film-forming vehicle not only imparts to such a vehicle the desired film strength, but also, as distinguished from gilsonite which some have heretofore thought to be its equivalent, does not absorb the taste and flavor of beverages, such as beer, but, on the contrary, insures their retention by the beverage over a long period.

In the accompanying drawing we have shown the invention applied to a container of the "tin can" type which is seamless, i. e., the top, body,

2

neck, and lip are drawn and formed from a single metal blank, e. g. black iron and are devoid of seams. The invention, however, is applicable to the lining of all types of containers, and in addition to metal cans, may be used upon paper receptacles as well as receptacles of plastics or synthetic materials.

In the drawing:

Figure 1 is a side elevation partly broken away, 10 showing our improved continuous lining applied to the container, and it is to be noted that the lining flows to such an extent as to cover a portion of the exposed surface of the sealing lip at the mouth of the container upon which the cork cushion of a cap such as the crown cap rests when the same is crimped upon the container;

Figure 2 illustrates the manner of applying wax to the can bottom, and

Figure 3 illustrates the manner in which the 20 wax drops are caused to flow into the bottom seam upon the lining so as to protect the seam against rusting, and fortify the seal.

The container shown in Figure 1 is formed of sheet metal, such as black iron or steel, and is 25 seamless, i. e., the body 10, top 11, neck 12, and sealing lip or cap receiving finish 13 are integral, being drawn from a single metal blank. The bottom 14 is convex, as shown, and is secured to the body 10 by seaming in the usual manner, as 30 shown at 15. The lining of the container is indicated at 16 and completely and continuously covers the interior wall of the container, including the bottom and the exposed flat top portion 17 of the lip upon which the cork cushion of a cap engages. The finish 13 in the present instance is of a type to receive a crown cap but other finishes may be used, if desired.

The lining 16 has the important characteristic of being non-absorbent and thereby preserves 40 the original quality and freshness of the most delicate foods and beverages. Furthermore, it is inert to the black iron of the container and to the beverage or food contents. In this respect it is advantageous over metallic coatings in which 45 electrolytic action may take place, leading to corrosion as well as objectionable effects upon the contents.

A composition suitable for a lining has for an 50 essential constituent a black bituminous resin known as "Aruba resin" purchasable in the open market, and preferably having a melting point of about 400° F. "Aruba resin" is a natural bituminous resin imported from the island of Aruba in Curacao, Dutch West Indies. The Wilson Carbon Company, New York city, markets this resin

under the name of "Vanadiset resin," the name being derived from the presence of a rare earth material in the resin, namely, approximately 0.25 percent of vanadium pentoxide ( $V_2O_5$ ). The resin contains about 25 percent of fixed carbon and the total elemental carbon of about 84.4% is in a colloidal form, and several percent of sulfur, but less than 0.5 percent of mineral matter. The resin is described by the seller as a crystalline form, readily pulverized, product of petroleum butane distillation and as a thermoplastic resin, which becomes plastic under treatment with heat. This "Aruba resin" is a black pitch contrasted to an asphalt which latter contains a much higher fixed carbon content, the range being 36 to 43 percent for Trinidad, Bermudez, Gilsonite, Tabylite, Wurtzelite, etc., (see Handbook of Chemical Engineering, vol. II, p. 647, by Liddell). The presence of 0.25 percent of vanadium pentoxide in "Aruba resin" is of value as a deoxidizing agent in the preservation of the film flexibility of varnishes made therefrom. The color of "Aruba resin" or "Vanadiset resin" is jet black, but brown when dissolved, and it is obtainable in grades melting at about 300° F. and 400° F. This 400° F. melting point "Aruba resin" is much higher than the melting points of the natural asphaltic resins, which in general melt below 300° F.

"Aruba" resin is a thermoplastic hydrocarbon compound containing vanadium pentoxide. It is also referred to as "Aruba" bitumen and as "Vanadiset" resin as above explained. The name "Vanadiset" resin has superseded "Aruba" resin in some cases since it is more expressive of the fact that this peculiar resin contains vanadium, which does not occur in any other known bitumen, and is believed to give it a high tensile strength without the elongation common to other pitch materials. The ash content (mineral matter) is about 0.5 percent, and it therefore contains little inorganic impurity.

An analysis of "Aruba" resin is as follows:

|                              | Percent |
|------------------------------|---------|
| Total carbon compounds       | 84.24   |
| Total fixed carbon           | 24.74   |
| Hydrogen                     | 8.53    |
| Nitrogen                     | 1.12    |
| Ash content (mineral matter) | 0.57    |
| $V_2O_5$                     | 0.25    |
| Water                        | 4.00    |
| Molecular weight             | 3200    |

The average moisture content of "Vanadiset" resin is 5.70 percent (as shipped), volatile matter (dry basis) 74.24 percent, fixed carbon 25.35 percent, ash .41 percent, vanadium oxide in ash 48.00 percent, melting point 300° F. to 400° F., specific gravity 1.117 at 60°, flash point 600-635° F.

By way of illustration, a preferred example has the following formula:

*Formula for black pitch coating*

|                    | Parts by weight |
|--------------------|-----------------|
| Aruba resin        | 84.0            |
| Rezyl resin #387-2 | 325.5           |
| W. W. kerosene     | 205.5           |
| Solvesso #3        | 120.0           |
| Total              | 735.0           |

Rezyl resin #387-2 is a short oil soya bean alkyd resin in solvent of the American Cyanamid Co. Kerosene is water white. Solvesso #3 is

an aromatic hydrocarbon solvent of the Standard Oil of New Jersey. Rezyl resin #387-2 contains about 50 percent resin and 50 percent of Solvesso #3 or its equivalent.

The 325-5 lbs. of #387-2 Rezyl resin is preferably mixed with the 120.0 lbs. of Solvesso #3 and the W. W. kerosene added. The whole is poured in ball mill, and the Aruba resin added, the whole being milled for a period long enough to disperse the Aruba resin throughout the vehicle.

Another formula on pounds and gallons basis, in which the weight proportion of resin and solvents is maintained as above, but the amount of Aruba resin is somewhat reduced is as follows:

|                    |              |
|--------------------|--------------|
| Aruba resin        | pounds 70    |
| Rezyl resin #387-2 | gallons 38.8 |
| Kerosene           | do 31.0      |
| Solvesso #3        | do 16.6      |

In a further example, this resin may be mixed with fuller's earth or volcanic clay, such as bentonite, together with a suitable plasticizer such as a reaction product between rosin and diethylene glycol or other plasticizer which, in its dry form, flows very sluggishly. The composition is carried in a solvent such as xylol or "Solvesso" sold by Standard Oil Company of New Jersey and is sprayed upon the container or the plate from which it is to be made. Thereafter, the sprayed coating is baked during which step the solvent is driven off and the coating is caused to flow so as to cover the exposed lip portion 17, and a thin continuous lining is produced which is non-absorbent. Such a protective coating on black plate will not be easily fractured. The coating is baked at a temperature of about 400° F. to 425° F. or above for a period of twenty minutes or more, the temperature being at or above the melting point of the resin ingredient, and a hard, dry, firm but flexible coating is produced.

Another lining is prepared by using a mixture of "Duraplex" resin and "Aruba resin." "Duraplex" resins are drying oil and non-drying oil "alkyd" resins, of which the products derived from phthalic anhydride, glycerine, and oil fatty acids may be considered the proto type. (This definition is taken from Duraplex bulletin of the Resinous Products & Chemical Co., Inc., Philadelphia, Pa.) A suitable resin is Duraplex C-49-S, which is a long oil drying type alkyd resin for air drying and baking finishes.

Below is a formula for the "Aruba resin" pitch coating including "Duraplex" resin:

|                 | Parts by weight |
|-----------------|-----------------|
| Aruba resin     | 300             |
| Bentonite       | 150             |
| Duraplex C-49-S | 450             |
| Solvent         | 1500            |

In preparing the coating 150 parts of bentonite are placed in a ball mill with 150 parts of solvent, e. g., a high boiling naphtha. After several hours of rotating the "Aruba resin" is added with 300 parts of additional solvent, and the rotating is continued for about 24 hours when "Duraplex" resin is added, with the remaining solvent. The rotation is continued for a few hours before the ball mill is emptied. The product is filtered and is ready for use as a spray. The composition should approximate 30 percent solids and 70 percent solvent. The preferred drying temperature on steel is between 400° F. and 425° F. for a time period of 20 minutes inside spray and 30 minutes outside spray.

As an addition in the preceding examples, we have satisfactorily used a composition containing an amorphoid wax, that is, a micro-crystalline paraffin wax, such as that refined from petrolatum. A melting point about 145° F. is preferred. Generally, these amorphoid waxes have melting points of 160° F. or above. If the wax is combined with a synthetic resin such as "Dura-pelix" resin, the wax is used in a relatively small amount, that is 2 to 3 percent of the total solids of the finished lining. The coating is baked at 400° F. to 425° F. The wax being of lower density than the "Aruba resin" and other solids in the composition has a tendency to bloom on the surface after baking. The wax is a particularly desirable ingredient in association with the "Aruba resin" since it is a flexifying agent for the lining film and is quite stable at the high baking temperatures, such as 400° F. or more. Moreover, the wax does not impart objectionable odors or taste in the baked sprayed coating and in addition to its stability at high baking temperature, also does not volatilize.

A further very efficient baked spray coating consists in preparing a mixture of plasticizing vehicle composed of bodied linseed oil 28 parts, manganese drier 2 parts, "Piccolyte resin" 17 parts, carnauba wax 3 parts, and solvent, such as xylene, 50 parts. Piccolyte resin is a chemical condensation polymer derived from B-pinene, which is in turn prepared from turpentine. To this mixture there is added 1½ pounds of "Aruba resin" to the gallon of vehicle and the resin and mixture are ground together preferably in a ball mill. The bodied linseed oil constitutes a plasticizing agent while the "Piccolyte resin" acts as a bonding agent and the carnauba wax is present as a reagent to self-lubricate the finished black lining.

Instead of the bodied linseed oil in the above formulation, we have used a product known as "G-80," of Ball Varnish Company, Pittsburgh, Pennsylvania. The "G-80" vehicle contains approximately 38 percent of total solids and 62 percent of solvent. The total solids contain resins suitably plasticized with drying oils, according to an analysis made of the product. Vehicles of a similar nature are obtainable on the market from numerous sources of supply.

A satisfactory lining has been prepared from the black bituminous resin sold under the trade name "Vanadiset," and the G-80 vehicle, by grinding the resin in the vehicle preferably by means of a ball mill. Approximately one pound of the resin is used to a gallon of the vehicle and the product is highly satisfactory to replace aluminum and other metal lining coatings.

In each of the examples heretofore described, it will be noted that these is provided a non-volatile and film-forming vehicle for the "Aruba" resin, and that this vehicle is present in substantially greater amount than the "Aruba." In other words, there is provided a varnish to which is added the "Aruba." We have discovered that "Aruba" does not have the objectionable flavor absorptive characteristics of gilsonite in the container lining art. It has, furthermore, been discovered that the "Aruba," even when present in substantially lesser amounts than varnish forming vehicles, such as synthetic resins, provides the characteristics desired and hereinbefore described.

While we have referred to the use of the compositions above mentioned as linings for metal containers, they are also satisfactory for paper

10  
15

coatings particularly those used as spotting materials in caps. For instance, a suitable paper coated with one of these linings will form a center spot facing or an overall facing for the closure cap. Also, closure caps such as crown caps may be formed from sheet metal provided on one or both sides with one of the coatings described above. The lining as a coating is advantageous over many lacquers because of its non-scratchability, resistance to rust, pasteurization, sterilization, etc., when applied to plain clean steel. It is unnecessary to bonderize, size, or otherwise treat the steel before its application. We prefer to use somewhat more resin and less solvent in the formula so as to body the material for coating instead of spray. It is also preferable to use a full pound or more of the Aruba resin to each gallon of vehicle.

While the present container lining has great flowability so that it flows out upon the exposed surface 17 of the lip of the container as well as into the joint defined by the seam 15 during baking, it is desirable to further fortify the bottom seam both against rusting and against leakage. It has been customary to use as linings for containers overall coatings of wax and this expensive procedure may be eliminated where the present lining is utilized. That is to say, the lining compositions described do not require the complete waxing of the interior wall of the can, and are highly receptive to wax coating so that the same may be applied over the lining at any particular spot or section.

Generally, this improved waxing procedure consists in passing the containers on a conveyor belt under fixed pipettes not shown, which place a drop or drops of wax 18 on the surface of the center of the convex container bottom, as shown in Figure 2. Thereafter, the containers are heated as by passing onto a hot plate 19 or heated section as shown in Figure 3, which melts or further disperses the wax in case the container is cold. Preferably, the container is pre-heated before the introduction of the wax. After the wax has been dropped, as shown in Figure 2, and the container subjected to heating, the wax runs over the convex inner surface of the bottom and into the joint, filling the crevices thereof as shown at 20 in Figure 3.

The possibility of the rust condition developing, which condition does not always appear very pronounced in a beer package but can be easily detected by analytical methods, is reduced to a minimum and as will be noted, it is only necessary to utilize the wax in the lower joint of the container.

The amount of wax required is negligible and depends on the size of the container, in that about 2½% to 25½% of a gram will be satisfactory for a 12 fl. oz. container or about ¼ of the 1.5 grams or more of wax required to completely coat the container.

A delicate product such as beer put up in containers constructed in this manner shows marked results, i. e., substantially the same satisfactory packaging obtained with glass containers. One of the great advantages of the lining as above pointed out is that it presents little danger of absorption of the aromatic principles of the beer such as the fine flavor of the esters in the beer, and since the wax is used in amount of only about 0.20 to 0.25 gram, it presents no absorption problem as is true where the whole interior wall of the container is wax coated.

As stated above, about 0.20 to 0.25 gram of wax

75

are satisfactory and may be applied as a single drop or a plurality of drops, e. g., 3 drops, 6 drops, or 8 drops.

A specific operation for applying the wax to the lower seam consists in melting the wax and maintaining the same in a suitable reservoir at a temperature of about 220° F. The reservoir is preferably in the form of a drip cup having at the bottom a T attachment with a nozzle and a valve, the nozzle having an aperture of  $\frac{1}{64}$  of an inch or slightly larger. When the valve is opened and the wax is dropped at the maximum rate of 120 drops per minute, it takes 6 to 8 drops to secure a protective coating on the inside seam. This is equivalent to about .195 to .260 gram of wax. Minimum protection can be had with 3 drops, equivalent to .096 gram per can but a slightly greater amount is preferred.

The drops of wax are dropped through the mouth of the can so that they fall upon the center of the inner convex surface as shown at 18 in Figure 2. The wax can be permitted to drop upon a cold surface but it is preferred that the bottom be pre-heated since in the subsequent heating step, the flow of the wax is much greater. After receiving the drops of wax, the cold or pre-heated containers are subjected to heat on the bottom as shown in Figure 3 at a temperature of about 250° to 280° F. When the cans are cold it takes possibly 10 to 15 seconds for the wax to properly distribute itself around a seam as shown at 20 in Figure 3, but when the containers are first warmed the distribution time of the wax can be substantially shortened to 5 to 10 seconds or less. The wax used has good flowing qualities and is one of those conventionally employed for container lining.

In applying the bituminous lining to the con-

ainers, the spraying is carried out with the containers upside down and with the bottom preferably attached, and the baking step is likewise conducted with the containers upside down, whereby sufficient flow of the lining is assured to provide a thoroughly protective coating film on the exposed surface 17 of the sealing lip continuous with the lining film on the interior wall and bottom of each container. When the waxing step is employed, the containers are in upright position and the wax dropped therein, as shown, upon the upwardly convex bottom.

The term "Aruba" resin as set forth in the appended claims is intended to cover a product having the physical and chemical properties set forth herein.

We claim:

1. A metal container having a lining in the form of a thin, continuous film comprising a major portion of film-forming resinous varnish having Aruba resin incorporated therein.

2. A metal container having a lining in the form of a thin, continuous film comprising a major portion of film-forming resinous varnish having Aruba resin with a melting point between 300° F. and 400° F. incorporated therein.

3. A metal container having a lining in the form of thin, continuous film comprising a major portion of film-forming resinous varnish having incorporated therein Aruba resin and wax.

4. A metal container having a lining in the form of a thin, continuous film comprising a major portion of film-forming resinous varnish having incorporated therein wax and Aruba resin having a melting point between 300° F. and 400° F.

ALBIN H. WARTH.  
ILIIYA F. BULATKIN.